

Dec. 22, 1931.

S. L. WILLIS

1,837,640

CONTAINER FOR GASOLINE

Filed Sept. 14, 1928



INVENTOR  
*Sanford L. Willis*  
BY  
*Dorey & Cole*  
ATTORNEYS.

## UNITED STATES PATENT OFFICE

SANFORD L. WILLIS, OF CORNING, NEW YORK, ASSIGNOR TO CORNING GLASS WORKS,  
OF CORNING, NEW YORK, A CORPORATION OF NEW YORK

## CONTAINER FOR GASOLINE

Application filed September 14, 1928. Serial No. 305,996.

This invention relates to dispensing containers and more particularly to transparent cylinders for containing gasoline and other fuels which are exposed to full view.

It is well known that gasoline, in the form in which it is offered to the public, varies from substantially a water white color to a noticeable yellow tint. There is also a general belief on the part of the public that the discoloredation of the gasoline is an indication of inferiority which, as a matter of fact, is not necessarily the case. It is also known that if certain grades of gasoline are exposed to the sunlight they acquire a yellow discoloredation.

I have discovered that this discoloredation of gasoline on exposure to sunlight can be prevented if the transparent container is made of ultra violet absorbing glass. I have also discovered that if such a glass is given a bluish hue it will mask the yellowish tint of certain kinds of gasoline and thus avoid creating the erroneous impression that such gasoline is of inferior quality.

It is therefore an object of my invention to prevent discoloredation of the gasoline contained in transparent dispensing cylinders.

Another object of my invention is to mask any inherent yellow coloration of the gasoline.

Still another object of my invention is to combine the above features in a glass which is both stable and workable.

With the above and other objects in view, which will be apparent as the description proceeds, I have set forth my invention in the following specification, taken in connection with the accompanying drawings, in which:

Fig. 1 is a side elevation of my improved gasoline cylinder embodied in a typical form of gasoline pump; and

Fig. 2 is a horizontal section through my gasoline cylinder on the line 2-2 of Fig. 1.

I have discovered that when gasoline is exposed to sunlight, decomposition will often occur and, in the case of certain types of gaso-

line this produces a white or pale yellow precipitate and a yellow color in the residual gasoline. I have also discovered that this decomposition and discoloration can be prevented if the container, through which the gasoline is exposed to sunlight, is made of ultra violet absorbing glass. Most ultra violet absorbing glasses, and especially those absorbing the ends of the visible spectrum, have a yellowish color or at least do not show a blue or other pleasing hue, since they absorb that part of the spectrum. Inasmuch as the purchasing public desires a water white gasoline, in the mistaken belief that a yellowish tint in the gasoline indicates that it is of inferior quality, the use of my new and improved gasoline cylinder prevents the decomposition of gasoline on exposure to sunlight and, owing to its bluish hue, disguises the objectionable yellow appearance of gasoline which has such a tint.

In the accompanying drawings, 10 designates a typical form of gasoline pump, provided with a body portion 11, a container supporting frame work 12, a top 13, an operating handle 14, and a container 15.

In carrying out my invention I made containers 15 for gasoline out of a transparent glass having substantial or complete absorption for the ultra violet rays. Glasses having the desired absorption are known in the art (although not used heretofore for the purpose stated) but I prefer to use as the glass from which the container is made one of the glasses described in the application of William C. Taylor, Serial No. 199,064, filed June 15, 1927, which not only possess the desired absorption characteristics, but also are capable of giving the contents a tint other than yellow or amber.

I disclose herein examples of the two types of glasses set forth in the application above mentioned, composition I being non-heat re-

60

65

75

80

85

85

85

85

85

85

85

85

85

85

85

85

85

85

sisting while composition II possesses heat resisting characteristics:

|                                      | I      | II     |
|--------------------------------------|--------|--------|
| 6                                    |        |        |
| SiO <sub>2</sub> .....               | 75     | 76.3   |
| Na <sub>2</sub> O.....               | 13.7   | 5.0    |
| K <sub>2</sub> O.....                | 2.0    | 2.1    |
| CaO.....                             | 2.0    |        |
| Al <sub>2</sub> O <sub>3</sub> ..... | 1.2    | 1.2    |
| B <sub>2</sub> O <sub>3</sub> .....  | 2.5    | 11.5   |
| 10 Rare earths.....                  | 3.6    | 3.8    |
| Co <sub>2</sub> O <sub>3</sub> ..... | Trace. | Trace. |

While I have found either of the above glass compositions to be admirably suited to my purpose, I recognize that there are various commercial glass compositions which may be adopted and successfully used in preventing the transmission of ultra violet rays to the gasoline, hence I do not limit myself to the specific glasses herein mentioned.

Having thus described my invention what I claim is:—

1. A transparent vending container for gasoline made of glass whose composition is such as to exclude substantially all of those ultra violet rays which discolor gasoline, said container furnishing and preserving visibility of the gasoline in its native color.

2. A vending container for gasoline made partially of transparent glass whose composition is such as to exclude substantially all of those ultra violet rays which discolor gasoline, the remainder of said container being made of such material that it also excludes said rays, the transparent portion of the container being designed to furnish and preserve visibility of the gasoline in its natural color.

SANFORD L. WILLIS.

40

45

50

55

60

65